

# United States Patent [19]

Culling

[11] Patent Number: 4,765,957

[45] Date of Patent: Aug. 23, 1988

[54] ALLOY RESISTANT TO SEAWATER AND OTHER CORROSIVE FLUIDS

[75] Inventor: John H. Culling, St. Louis, Mo.

[73] Assignee: Carondelet Foundry Company, St. Louis, Mo.

[21] Appl. No.: 947,095

[22] Filed: Dec. 29, 1986

[51] Int. Cl.<sup>4</sup> ..... C22C 30/02

[52] U.S. Cl. ..... 420/582; 420/584; 420/585; 420/586

[58] Field of Search ..... 420/45, 46, 47, 584, 420/582, 585, 586

## [56] References Cited

### FOREIGN PATENT DOCUMENTS

57-16153 1/1982 Japan ..... 420/45  
1142582 2/1969 United Kingdom ..... 420/45

Primary Examiner—Deborah Yee

Attorney, Agent, or Firm—Senniger, Powers, Leavitt and Roedel

[57]

## ABSTRACT

The alloys of this invention are of low strategic element content, nonmagnetic, resistant to damage by chloride- or other halide-containing solutions as well as to a wide variety of other chemical agents, airmelttable, castable, of improved fabricability and weldability and of higher chromium level but lower molybdenum contents than other alloys intended for chloride resistance. The alloys consist by weight percentages of from about 13.5% to about 29% Ni, from about 23 to about 26% Cr, from about 3.75 to about 6% Mo, from about 2.95 to about 4.5% Mn, from about 3 to about 6.39% Cu, from about 0.3 to about 2.07% Cb (Nb), from about 0 to about 1.5% Si, from about 0 to about 0.09% C, from about 0.10% to about 0.45% N, up to about 1% V, up to about 1% Ti, up to about 5% Co, as a partial substitute for Ni, up to about 0.3% Ce, La or Misch metal, and the balance essentially iron. The sum of the Ni and Co content is between about 18.5% and about 29% by weight.

5 Claims, 1 Drawing Sheet





## ALLOY RESISTANT TO SEAWATER AND OTHER CORROSIVE FLUIDS

### BACKGROUND OF THE INVENTION

There is great demand for materials resistant to sea water, brackish water or other solutions that contain chlorides or other halide ions. Examples are equipment for surface vessels and submarines and for various chemical handling and power plant applications.

At the present time the two most important known elements that confer chloride resistance to iron-base or nickel-base alloys are molybdenum and chromium.

For maritime application, an alloy has been considered generally satisfactory if it resists corrosion by seawater at ambient temperatures. Recently, however, the extensive use of seawater or brackish water as a cooling medium in heat exchangers has increased, with the result that there is great demand for materials that resist damage by both seawater and the process fluids that are being cooled. In some cases, the process fluid is highly corrosive to many materials, even to some that are able to resist seawater attack. Much progress has been made in developing materials with the required corrosion resistance and other properties. However, such materials have tended to be quite expensive, high in critical or strategic element content, and difficult to prepare and fabricate. Thus, there is great interest in the development of lower cost alloys that are more effective or more efficient than those presently in service in resisting attack by seawater and process fluids.

There is also the desirability in some applications that such alloys be substantially nonmagnetic. One such application is for naval mine-sweepers which must avoid destruction by magnetic mines. Nonmagnetic alloys are also advantageous materials of construction for submarines, since they allow the vessel to elude the magnetic anomaly detector systems that are employed to locate submerged submarines. These systems sense changes in the earth's magnetic field caused by metallic masses as large as steel submarines.

The element titanium and its principal alloys are nonmagnetic, are totally immune to ordinary seawater attack, and have been employed in the hulls of a few submarines and in the heat exchanger tubes of a few seawater-cooled power plants. However, titanium is relatively scarce and expensive, quite difficult to fabricate, and very susceptible to contamination and embrittlement if processed by conventional methods. Hence, Ti weldments tend to crack and leak, and Ti cannot be melted and cast into shapes except under the most rigorous conditions in vacuum or inert gas atmospheres. Also, use of titanium tubing in retrofitting existing heat exchangers may lead to excessive vibration failures unless dampeners are used or support sheets are repositioned.

Thus, there is continued interest in air melttable, castable, weldable, fabricable alloys to resist attack by sea water, and for many applications that remain essentially non-magnetic.

In spite of their excellent overall corrosion resistance, the usual commercial stainless steels are subject to localized corrosion in stagnant seawater. Stagnant conditions arise when the flow rate over the metallic surfaces is less than about 1.2 to 1.6 meters per second (3.9 to 5.2 feet per second), when marine organisms are attached to the surfaces, or where crevices exist. Such conditions are very difficult to avoid completely in actual practice.

Thus, although general corrosion of stainless steel components tends to be very low in seawater, very serious damage leading to early failure often occurs because of localized corrosion.

5 Pitting attack and penetration or perforation of stainless steels tend to take place on broad surfaces with low fluid flow rates, while some form of crevice corrosion takes place where there are imperfect contacts with mud, fouling substances, wood, paint, or other bodies, or even where there are reentrant angles or corners.

10 A major obstacle to the use of austenitic stainless steels for service in strong chloride environments has been the possibility of chloride stress corrosion cracking. Under conditions of even moderate stress and temperature, type 304 (ordinary 18% Cr 8% Ni) stainless steel will crack at very low chloride levels. Stress corrosion cracking has not really been well understood in the past, but it is now known that improved and highly modified stainless steels of higher molybdenum contents 15 above 3.5% have a degree of resistance to chloride stress corrosion cracking that is more than adequate for most high chloride service.

15 Ferritic iron-chromium-molybdenum stainless steels have been developed for chloride service, but they must be produced with extremely low carbon and nitrogen contents, and are hence not available as cast shapes by ordinary production methods. They are also magnetic and readily attacked by many common chemicals.

20 25 30 35 A number of austenitic, nonmagnetic, nickel-base alloys have also been developed for the same types of service. These have contained up to 31% Cr, up to 28% Mo, and from about 45% to about 65% Ni. They often contain 1 to 4% W and up to 4% Cb (Nb) plus Ta, iron being limited to levels around 2 to 6% maximum. The combined proportion of Mo, Cr and W in these alloys varies between about 32 and 42% total. Such high levels of the latter elements require very high nickel and low iron contents in order to maintain a single-phase austenitic (face-centered-cubic) crystal structure. While these nickel-base alloys are castable, weldable, and fairly 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 99

where. "Sour" means that the fluids are high in hydrogen sulfide and mercaptan contents. In addition to sulfur compounds, deep sour wells also encounter carbon dioxide, salts such as brine, and temperatures up to 300° to 500° F. (150° to 260° C.). These are all examples of severe service conditions in which chloride resistance of my prior alloy or of the usual commercial chloride-resistant alloys may not be adequate.

#### SUMMARY OF THE INVENTION

Among the several objects of the present invention, therefore, may be noted the provision of improved alloys resistant to chlorides as well as other corrosive streams; the provision of such alloys which are resistant to process streams of corrosive fluids such as may be encountered in heat exchangers and process equipment used in the manufacture or handling of contaminated phosphoric acid, various concentrations of hot sulfuric acid, and deep sour well fluids; the provision of such alloys which may be economically formulated with relatively low proportions of strategic metals such as nickel, chromium and molybdenum; the provision of such alloys whose strategic metal content is sufficiently low so that they may be formulated from such relatively low-cost raw materials as scraps, ferro alloys or other commercial melting alloys; the provision of such alloys which can be cast or wrought; the provision of such alloys which have a low hardness and high ductility so that they may be readily rolled, forged, welded and machined; the provision of such alloys which are air-meltalbe and air-castable; the provision of such alloys which are substantially nonmagnetic, i.e., for military and naval applications such as minesweepers and submarines; the provision of such alloys that do not require heat treatment after welding or hot working to avoid intergranular attack; the provision of such alloys which resist pitting attack, crevice corrosion and stress corrosion cracking failures; and the provision of such alloys which are resistant to localized attack in stagnant seawater.

Briefly, therefore, the present invention is directed to an air-meltalbe, castable, workable, non-magnetic alloy resistant to corrosion by chloride-containing solutions. The alloy consists essentially of between about 13.5% and about 29% Ni, from about 23% to about 26% Cr, from about 3.75% to about 6% Mo, from about 3% to about 4.5% Mn, from about 3% to about 6.39% Cu, from about 0.10% to 0.45% N, from about 0.3% to about 2.07% Cb, up to about 1.5% Si, up to about 0.09% C, up to about 1% Ti, up to about 5% Co as a partial substitute for Ni, and up to about 0.3% Ce, La or misch metal. All of the above percentages are by weight. The sum of the Ni content and Co content is between about 18.5% and about 29% by weight.

#### BRIEF DESCRIPTION OF THE DRAWING

The single FIGURE of the drawing is a plot of an algorithm useful in formulating alloys resistant to chloride stress corrosion cracking.

#### DESCRIPTION OF THE PREFERRED EMBODIMENT

In accordance with the present invention, alloys are provided which are virtually immune to chloride or sea water depassivation and are at the same time very highly resistant to the attack of certain corrosive chemical process streams. In particular, it has been found that the alloys of the invention are effective materials of

construction for process equipment exposed to process fluids such as those encountered in the manufacture of phosphoric acid, and in the recovery of sour gas and oil from off-shore wells. These alloys have further been demonstrated to be effective in resisting corrosion by both pure and impure sulfuric acid solutions over a wide range of concentrations.

The alloys, in part because of their higher chromium content, resist the corrosive attack of many chemical agents not successfully resisted by prior lower chromium commercial alloys.

Resistance to crevice corrosion and to corrosion under stagnant or low flow conditions are particular advantages of the alloys of the invention when used in seawater or other high chloride solutions. Thus, mud, fouling substances, paint and similar materials do not induce corrosion when imperfectly coated on alloys of the invention exposed to a seawater environment. Additionally, the alloys are non-magnetic and useful for surface and submarine vessel hull construction.

The alloys of the invention are air-meltalbe and air-castable and possess advantageous mechanical properties which render them suitable as materials of construction for tanks, tubes, pipes, plates, pressure vessels, pumps, agitators, valves, tube sheets and supports for heat exchangers, and cleats, stanchions, pulleys, and deck fittings for oceangoing vessels, off-shore oil and gas rigs, docks and deep "sour" gas and oil drilling and pumping equipment. More particularly, the alloys of the invention are ductile, and thus may be wrought into forms suitable for the above applications.

Unlike the nickel-base alloys which have been used for such service, the alloys of the present invention can be formulated from ferro-alloys, scraps and commercial melting alloys, sources which may contain impurities or contaminants not permitted in nickel-base alloys.

The chromium levels of the alloys of this invention have been recognized for many years to have great advantage in many types of service over those alloys of the 15 to 21% Cr levels. The alloys of the present invention have been so formulated as to take advantage of this and yet at the same time maintain resistance to chloride depassivation.

The nickel levels in the alloys of this invention are such as to maintain a single phase, austenitic (face-centered-cubic) crystal structure in conjunction with the manganese and nitrogen contents. Other prior art alloys have often employed considerably lower nickel levels to the detriment of corrosion resistance in many substances. On the other hand the very high nickel levels of the nickel-base alloys have not been found necessary for most corrosion situations.

Manganese is also a weak austenite stabilizer and is so employed in the alloys of the present invention. However, Mn is also beneficial in increasing resistance to chloride depassivation.

Nitrogen is similar to Mn in the alloys of the present invention. The main difference is that nitrogen, on a weight percent basis, is very much more effective as an austenite stabilizer and in increasing chloride resistance than is Mn. However, nitrogen is a gas in its natural state and must not exceed the maximum of about 0.45% in these alloys if porosity is to be avoided in production. Fontana, U.S. Pat. No. 2,214,128, claims 1% to 4% Mn in iron-nickel-chromium molybdenum-copper alloys. Fontana states that Mn, when added in the proportions as set forth, adds to the alloy the quality of ease of fabrication and does not detract from the corrosion

resistance of the alloy. In fact, Fontana illustrates only one example of his invention, namely about 26.7% Ni, 19.7% Cr, 3.4% Mo, 2.0% Cu, and 2.080% Mn. The alloys of the present invention are believed to be effective in part due to higher Cr, Mo and Mn levels than Fontana's one example. The Mn level in Fontana's single example was not high enough to present any of the advantages of Mn in the 3 to 4% range. The level of Mn in the present invention is sufficiently high to aid in chloride resistance, to help stabilize a single-phase austenitic metallic structure and to increase solubility of nitrogen in the solid metallic alloy.

Copper broadens the useful range of chemical solutions to which the alloy is resistant, and enhances the resistance of these alloys to particular solutions without the detriment to chloride resistance often reported by other workers in the field.

Silicon is limited to a maximum of about 1.5% by weight in alloys of this invention so as not to damage their fabricability or weldability. Except for this factor higher Si levels would normally be tolerated in most solutions. Because Mn is such a strong deoxidizer, the very low Si levels that may be allowed in alloys of this invention are of no consequence in maintaining cleanliness and soundness of castings and ingots, although Si is intentionally added in many low Mn alloys for the purpose of deoxidation.

Cerium, lanthanum, misch metal, or some combination of rare earth elements may be arbitrarily added in amounts less than 1% for the purpose of improving workability of ingots of these alloys according to the principles set forth by Post, et. al., U.S. Pat. No. 2,553,330.

Vanadium also enhances the resistance of these alloys to chlorides and acts as a grain refiner. It has been found to be of benefit in amounts up to 1% in alloys of this invention and may be so added without detriment to chemical resistance.

Cobalt may be partially substituted for Ni up to 5% Co without detriment and is sometimes found in Ni-containing ores. Cobalt may thus be regarded in the same manner as Ni in these quantities.

Columbium (niobium) is also employed in alloys of this invention to help resist general chemical attack and as a carbide stabilizer against intergranular corrosion. It has been found to beneficially enhance corrosion resistance of alloys of this invention in amounts up to about 2%.

Combinations of Cr and Mo within the range of proportions of the invention contribute significantly to the resistance of those alloys against attack by seawater. Moreover, where the combination of Cr and Mo satisfies the preferred relationship

$$[\text{Mo}] \geq \frac{31}{[\text{Cr}] - 12} + 2$$

where

$[\text{Mo}]$  = weight % molybdenum and

$[\text{Cr}]$  = weight % chromium.

it has been found that the alloys of the invention are especially resistant to  $\text{Cl}^-$  stress corrosion cracking, as well as  $\text{Cl}^-$  pitting. A plot of this algorithm is set forth in the drawing. Alloys having a combination of Cr and Mo falling above and/or to the right of the curve have been found to exhibit effective resistance to stress corrosion cracking.

Tantalum sometimes occurs in ores along with columbium and may be present in alloys of the invention

without detriment up to about  $\frac{1}{2}$  of the columbium content.

Carbon has been tested in alloys of the invention to 0.11% without intergranular corrosion if the other element contents are adjusted. Normally, however, it is desirable to maintain carbon levels below about 0.08%.

The essential components of the invention are:

|    |            |                    |
|----|------------|--------------------|
| 10 | Nickel     | 13.5-29% by weight |
|    | Chromium   | 23-26%             |
|    | Molybdenum | 3.75-6%            |
|    | Copper     | 3.0-6.39%          |
|    | Manganese  | 2.95-4.5%          |
| 15 | Columbium  | 0.3-2.07%          |
|    | Nitrogen   | 0.10-0.45%         |
|    | Iron       | 28-48%             |

Cobalt may be present in a proportion of up to about 5% by weight as a partial substitute for Nickel. In any case, the sum of the cobalt and nickel contents should range between about 18.5% and about 29% by weight.

Normally, the alloys of the invention will also contain carbon, up to a maximum of about 0.08% by weight.

Optionally, the alloys of the invention may further contain:

|    |                                  |            |
|----|----------------------------------|------------|
| 30 | Silicon                          | Up to 1.5% |
|    | Titanium                         | Up to 1%   |
|    | Vanadium                         | Up to 1%   |
|    | Tantalum                         | Up to 1%   |
|    | Cerium, Lanthanum or Misch Metal | Up to 0.3% |

While many chemical conditions may be well served by alloys containing nickel at the lowest levels of this invention, there are other conditions, including some ranges of sulfuric acid concentration, in which the nickel contents of alloys of the invention should exceed the corresponding chromium contents by at least about 0.5% but not more than about 6% (basis, the entire alloy).

Also, certain conditions are better met with copper contents toward the low side of the above specified ranges. Hence, in many corrosion situations, it has been found preferable to restrict the proportions of the component elements to the following ranges:

|    |                       |                                  |
|----|-----------------------|----------------------------------|
| 50 | Nickel                | 24-29%                           |
|    | Chromium              | 23-26%                           |
|    | Molybdenum            | 3.75-6%                          |
|    | Copper                | 3-4.5%                           |
|    | Manganese             | 2.95-4.5%                        |
|    | Columbium             | 0.3-2.07%                        |
|    | Nitrogen              | 0.10-0.45%                       |
| 55 | Silicon               | 0.10-0.50%                       |
|    | Carbon                | 0.05% Maximum                    |
|    | Nickel minus Chromium | 0.5-6% (basis, the entire alloy) |

While columbium enhances resistance to some corrosive streams, its most effective range in alloys of the invention lies between about 0.3 and about 1.5% by weight. Also, the most effective range of nitrogen in alloys of the invention is between about 0.10 and about 0.25%. For even better resistance to the widest range of corrosive conditions the components of the alloys of this invention should be even further restricted to the following ranges of proportions:

TABLE II

|                       |                                |
|-----------------------|--------------------------------|
| Nickel                | 25-29%                         |
| Chromium              | 23-26%                         |
| Molybdenum            | 4-6%                           |
| Copper                | 3-4.5%                         |
| Manganese             | 2.95-4.5%                      |
| Columbium             | 0.3-1.5%                       |
| Nitrogen              | 0.10-0.25%                     |
| Nickel minus Chromium | 2-5% (basis, the entire alloy) |

In an especially preferred embodiment of the invention the nickel content of the alloy exceeds the chromium content by about 3 to about 5% with other components in the following ranges of proportions:

|                       |                                |
|-----------------------|--------------------------------|
| Nickel                | 26-29%                         |
| Chromium              | 23-26%                         |
| Molybdenum            | 4.5-5.5%                       |
| Copper                | 3-4%                           |
| Manganese             | 3-4%                           |
| Columbium             | 0.5-1.0%                       |
| Nitrogen              | 0.15-0.25%                     |
| Carbon                | 0.01-0.04%                     |
| Silicon               | 0.10-0.40%                     |
| Nickel minus Chromium | 3-5% (basis, the entire alloy) |

A particularly advantageous alloy having optimum properties in various services combined with optimum mechanical properties has the following composition:

|            |       |
|------------|-------|
| Nickel     | 27%   |
| Chromium   | 23%   |
| Molybdenum | 5%    |
| Copper     | 3%    |
| Manganese  | 3.5%  |
| Columbium  | 0.8%  |
| Nitrogen   | 0.20% |
| Silicon    | 0.30% |
| Carbon     | 0.03% |
| Iron       | 35%   |

The following examples illustrate the invention.

#### EXAMPLE 1

One hundred pound heats of several different alloys were prepared in accordance with the invention. Each of the heats was air-melted in a 100-pound high frequency induction furnace. The composition of these alloys is set forth in Table I with the balance in each instance being essentially iron.

TABLE I

#### PERCENT BY WEIGHT OF ALLOYING ELEMENTS

| ALLOY NO. | Ni    | Cr    | Mo   | Cu   | Mn   | Si  | C   | Cb   | Others |
|-----------|-------|-------|------|------|------|-----|-----|------|--------|
| 1411      | 21.52 | 23.44 | 5.27 | 3.07 | 3.42 | .29 | .02 | .31  | .21    |
| 2215      | 25.43 | 24.87 | 4.30 | 3.50 | 3.74 | .25 | .04 | .43  | .18    |
| 2216      | 26.34 | 25.87 | 3.93 | 3.50 | 2.95 | .29 | .05 | .40  | .43    |
| 2224      | 25.38 | 25.02 | 3.88 | 6.39 | 3.26 | .57 | .05 | .61  | .34    |
| 2234      | 27.20 | 23.07 | 3.77 | 3.11 | 3.64 | .58 | .05 | 1.95 | .27    |
| 2235      | 27.65 | 23.95 | 5.62 | 3.23 | 4.26 | .48 | .08 | 2.07 | .31    |
| 2331      | 25.37 | 23.88 | 5.05 | 3.16 | 3.50 | .28 | .03 | .81  | .20    |
| 2226      | 28.59 | 23.02 | 4.73 | 3.50 | 3.83 | .44 | .05 | 1.58 | .12    |

Standard physical test blocks and corrosion test bars were prepared from each heat. Using the as-cast non-heat-treated physical test blocks, the mechanical properties of each of these alloys were then measured. The results of these measurements are set forth in Table II.

| ALLOY NUMBER | TENSILE STRENGTH P.S.I. | YIELD STRENGTH P.S.I. | TENSILE ELONGATION % | PHYSICAL PROPERTIES OF ALLOYS AS CAST |  |
|--------------|-------------------------|-----------------------|----------------------|---------------------------------------|--|
|              |                         |                       |                      | BRINELL HARDNESS NUMBER               |  |
| 1411         | 53,000                  | 30,800                | 16.2                 | 153                                   |  |
| 2215         | 74,700                  | 46,800                | 22                   | 181                                   |  |
| 2216         | 63,300                  | 36,600                | 19                   | 160                                   |  |
| 2224         | 70,600                  | 44,900                | 21                   | 173                                   |  |
| 2234         | 55,300                  | 31,800                | 12.5                 | 137                                   |  |
| 2235         | 57,500                  | 37,900                | 7.5                  | 170                                   |  |
| 2331         | 75,400                  | 47,600                | 20                   | 179                                   |  |
| 2226         | 53,200                  | 31,500                | 16.5                 | 137                                   |  |

Without heat treatment, the corrosion test bars were machined into 1½ inch diameter by ¼ inch thick discs, each having a ½ inch diameter hole in the center.

These discs we used in the comparative corrosion tests, described hereinafter, comparing the performance of the alloys of the invention with a number of alloys which either conform to the prior art or which are similar to the alloys of this invention but do not satisfy certain of the critical composition limitations of the alloys of the invention. The compositions of the comparative alloys used in the tests are set forth in Table III.

| ALLOY NUMBER | PERCENTAGE BY WEIGHT OF ALLOYING ELEMENTS |       |       |      |      |     |     |    |
|--------------|-------------------------------------------|-------|-------|------|------|-----|-----|----|
|              | Ni                                        | Cr    | Mo    | Cu   | Mn   | Si  | C   | Cb |
| 2396         | 18.73                                     | 18.30 | 6.39  | 1.16 | 3.78 | .32 | .03 | —  |
| 254SMO       | 18.86                                     | 20.86 | 6.15  | .81  | .51  | .24 | .01 | —  |
| VEWA963      | 16.15                                     | 17.01 | 6.31  | 1.57 | .77  | .58 | .02 | —  |
| IN862        | 24.22                                     | 21.12 | 5.08  | —    | —    | —   | .02 | —  |
| 1399         | 19.02                                     | 17.69 | 7.86  | .68  | 3.84 | .31 | .01 | —  |
| 1405         | 19.41                                     | 18.67 | 6.80  | 1.40 | 3.62 | .14 | .01 | —  |
| 1406         | 15.07                                     | 14.64 | 18.34 | 1.41 | 3.19 | .26 | .02 | —  |
| 1407         | 15.27                                     | 17.24 | 6.90  | 1.70 | 3.35 | .25 | .01 | —  |
| 1398         | 19.75                                     | 17.93 | 7.49  | .87  | 3.36 | .26 | .01 | —  |
| AL6X         | 24.20                                     | 20.12 | 6.24  | —    | .66  | .55 | .02 | —  |
| 316          | 13.11                                     | 17.92 | 2.46  | —    | .89  | .66 | .03 | —  |

Test discs from alloys of this invention along with those from the various comparative alloys were placed in about 1½" depth of salt solution in plastic containers fitted with virtually airtight lids. The solution consisted of 4 ounces of ordinary, uniodized table salt per gallon of ordinary St. Louis, Mo. city tap water. Twenty-five samples were in each container. They were not touching each other or any other metal—only the bottom of the container.

The liquid from each container was siphoned off once every seven days and replaced by freshly prepared salt solution. The top surfaces of all discs were examined for the appearance of pits or rust spots, which first appeared as reddish-colored spots.

After 160 days of exposure at ambient temperatures the discs were then washed and dried and examined at a magnification of 20× for evidence of pitting or local corrosion on the top surfaces as well as on the bottom surfaces, which had remained in close, stagnant contact with the surface of the plastic containers for the 160 days.

The first appearance of rust spots were as follows: 254SMO—79 days, VEWA963—55 days, IN862—48 days, 1406—84 days, 1407—55 days, Type 316 Stainless Steel—3 hours. No rust spots had appeared on the top

or bottom surfaces of any of the alloys of this invention or upon 1399, 1405 or 2396.

### EXAMPLE 2

A test similar to that of Example 1 was run on test discs from all of the above alloys of Example 1. In the test of this example, the plastic containers were filled with 4 ounces of salt per gallon of distilled water plus 4% nitric acid. The pH, or acidity, of this solution was measured at 2.0. It has been shown by many workers in the field of sea water corrosion that decreasing the pH, i.e., increasing hydrogen ion concentration and activity, of a chloride solution causes that solution to more readily depassivate stainless steels and similar alloys. Alloys with resistance to lower values of depassivation pH exhibit better resist crevice corrosion or pitting under stagnant conditions.

In this test, the samples were removed, washed, dried and examined at a magnification of 20 $\times$  after 60 days exposure. The alloys of this invention were found to have no visible pits or penetration, although alloys 2215, 2216, and 2224 showed small areas of very faint rainbowcolored stains.

All of the other samples not of this invention displayed various amounts of local attack in the form of small black spots of deep penetration on the bottom faces and various sized areas of clear metallic color on the top and bottom faces of the discs. These areas appear as a relatively shallow attack that selectively etches the crystalline dendritic pattern.

### EXAMPLE 3

Test discs of alloys of this invention were suspended by platinum wires in 10%, 25%, 40% and 97% sulfuric acid-water solutions at 80° C. (176° F.). Test discs of comparative alloys were also tested in these solutions. The test discs were measured to the nearest 10,000th of a gram before and after exposure and the weight loss expressed in inches per year,  $R_{ipy}$ , in accordance with this relationship:

$$R_{ipy} = 0.3937 \frac{W_o - W_f}{ATD}$$

$R_{ipy}$ =Corrosion rate in inches per year

$W_o$ =Original weight of sample

$W_f$ =Final weight of sample

$A$ =Area of sample in square centimeters

$T$ =Duration of test in years

$D$ =Density of alloy in grams per cubic centimeter

The tests were run for a total of six days exposure. The results are set forth in Table IV.

### TABLE IV

CORROSION RATE IN INCHES OF PENETRATION PER YEAR (I.P.Y.) AT 80° C. IN VARIOUS SULFURIC ACID-WATER SOLUTIONS

| ALLOY NUMBER | 10% BY H <sub>2</sub> SO <sub>4</sub> | 25% BY H <sub>2</sub> SO <sub>4</sub> | 40% BY H <sub>2</sub> SO <sub>4</sub> | 97% BY H <sub>2</sub> SO <sub>4</sub> |
|--------------|---------------------------------------|---------------------------------------|---------------------------------------|---------------------------------------|
| 1411         | 0.0003                                | 0.0006                                | 0.0850                                | 0.0197                                |
| 2215         | 0.0018                                | 0.0026                                | 0.0275                                | 0.0083                                |
| 2216         | 0.0041                                | 0.0034                                | 0.0235                                | 0.0054                                |
| 2224         | 0.0014                                | 0.0030                                | 0.0338                                | 0.0078                                |
| 2226         | 0.0022                                | 0.0030                                | 0.0135                                | 0.0076                                |
| 2234         | 0.0010                                | 0.0025                                | 0.0169                                | 0.0054                                |
| 2235         | 0.0029                                | 0.0000                                | 0.0229                                | 0.0066                                |
| 2331         | 0.0008                                | 0.0015                                | 0.0000                                | 0.0039                                |
| 254SMO       | 0.0108                                | 0.0064                                | 0.0751                                | 0.0178                                |

TABLE IV-continued

CORROSION RATE IN INCHES OF PENETRATION PER YEAR (I.P.Y.) AT 80° C. IN VARIOUS SULFURIC ACID-WATER SOLUTIONS

| ALLOY NUMBER | 10% BY H <sub>2</sub> SO <sub>4</sub> | 25% BY H <sub>2</sub> SO <sub>4</sub> | 40% BY H <sub>2</sub> SO <sub>4</sub> | 97% BY H <sub>2</sub> SO <sub>4</sub> |
|--------------|---------------------------------------|---------------------------------------|---------------------------------------|---------------------------------------|
| VEWA963      | 0.0259                                | 0.0163                                | 0.0667                                | 0.0061                                |
| IN862        | 0.0022                                | 0.0030                                | 0.0135                                | 0.0075                                |
| 2396         | 0.0133                                | 0.0029                                | 0.0673                                | 0.1550                                |
| 1399         | 0.0115                                | 0.0083                                | 0.0383                                | 0.0136                                |
| 1405         | 0.0191                                | 0.0035                                | 0.0595                                | 0.0212                                |
| 1406         | 0.1720                                | 0.0168                                | 0.0189                                | 0.0059                                |
| 1407         | 0.0646                                | 0.0627                                | 0.0688                                | 0.0062                                |
| 1398         | 0.0073                                | 0.0047                                | 0.0326                                | 0.0056                                |
| AL6X         | 0.0061                                | 0.0092                                | 0.0102                                | 0.0431                                |
| 316          | 0.0131                                | 0.0711                                | 0.2133                                | 0.0071                                |

Although there are applications in which higher corrosion rates may be tolerated, about 0.01 I.P.Y. may be considered as a practical maximum for most applications. It is obvious that the alloys of this invention are suitable in the reducing end of the sulfuric acid-water range up to 25% H<sub>2</sub>SO<sub>4</sub> but generally not suitable to 40% H<sub>2</sub>SO<sub>4</sub>. They also handle the oxidizing 97% H<sub>2</sub>SO<sub>4</sub> solution. Most of the alloys not of this invention are not usable in the 10 to 25% range and many will not endure the 97% solution.

### EXAMPLE 4

Test discs of the invention along with comparative samples of alloys not of this invention were tested for six days at 80° C. (176° F.) in 35% nitric acid-water solution as well as in the same acid concentration to which 4 ounces per gallon of sodium chloride were also added as a chloride depassivator. The results are set forth in Table V.

TABLE V

CORROSION RATE INCHES OF PENETRATION PER YEAR (I.P.Y.) AT 80° C. IN 35% NITRIC ACID-WATER SOLUTION, WITH AND WITHOUT 4 OZ./GAL. SALT ADDITION

| ALLOY NUMBER | 35% BY WEIGHT HNO <sub>3</sub> | 35% BY WEIGHT HNO <sub>3</sub> + 4 OZ./GAL. NaCl |
|--------------|--------------------------------|--------------------------------------------------|
| 1411         | 0.0023                         | 0.0018                                           |
| 2215         | 0.0014                         | 0.0041                                           |
| 2216         | 0.0013                         | 0.0004                                           |
| 2226         | 0.0000                         | 0.0006                                           |
| 2234         | 0.0027                         | 0.0004                                           |
| 2235         | 0.0036                         | 0.0016                                           |
| 2331         | 0.0007                         | 0.0013                                           |
| 254SMO       | 0.0015                         | 0.0027                                           |
| VEWA963      | 0.0020                         | 0.0111                                           |
| IN862        | 0.0000                         | 0.0004                                           |
| 2396         | 0.0000                         | 0.0047                                           |
| 1399         | 0.0036                         | 0.0127                                           |
| 1405         | 0.0014                         | 0.0210                                           |
| 1406         | 0.0063                         | 0.1052                                           |
| 1407         | 0.0020                         | 0.0113                                           |
| 1398         | 0.0011                         | 0.0078                                           |

From this test it may be seen that even the low-chromium alloys readily passivate in the very highly oxidizing hot 35% nitric acid solution. However, among the comparative alloys even those of high-molybdenum contents do not always maintain passivity in the same acid which also contains the chloride contamination.

On the other hand, the alloys of this invention were not depassivated by the chloride additions to the nitric acid.

## EXAMPLE 5

Test discs of alloys of the invention along with comparative samples of other alloys were then tested for six days at 80° C. (176° F.) in 86% phosphoric acid to which had been added 4 ounces per gallon of ordinary table salt. The results are set forth in Table VI.

TABLE VI

| ALLOY NUMBER | CORROSION RATE AT 80° C. IN 86% H <sub>3</sub> PO <sub>4</sub> PLUS 4 OZ. PER GALLON OF NaCl | LOSS IN INCHES OF PENETRATION PER YEAR (I.P.Y.) |
|--------------|----------------------------------------------------------------------------------------------|-------------------------------------------------|
|              | LOSS IN INCHES OF PENETRATION PER YEAR (I.P.Y.)                                              |                                                 |
| 1411         | 0.0028                                                                                       |                                                 |
| 2215         | 0.0034                                                                                       |                                                 |
| 2216         | 0.0036                                                                                       |                                                 |
| 2226         | 0.0092                                                                                       |                                                 |
| 2234         | 0.0014                                                                                       |                                                 |
| 2235         | 0.0022                                                                                       |                                                 |
| 2331         | 0.0016                                                                                       |                                                 |
| 254SMO       | 0.0244                                                                                       |                                                 |
| VEWA963      | 0.0507                                                                                       |                                                 |
| IN862        | 0.0095                                                                                       |                                                 |
| 2396         | 0.0080                                                                                       |                                                 |
| 1399         | 0.0182                                                                                       |                                                 |
| 1405         | 0.0253                                                                                       |                                                 |
| 1406         | 0.0243                                                                                       |                                                 |
| 1407         | 0.0509                                                                                       |                                                 |
| 1398         | 0.0098                                                                                       |                                                 |

This example is one of a moderately aggressive reducing condition plus depassivating chloride contamination.

The alloys of this invention serve very well here, while the lower chromium prior art alloys are either borderline or unsuitable.

Alloys of this invention also resist moderately aggressive oxidizing agents, such as 97% H<sub>2</sub>SO<sub>4</sub> much better than most prior art sea water alloys. They share excellent resistance with the prior art alloys to very aggressive oxidizing agents such as hot 35% HNO<sub>3</sub>, with or without chloride contamination. All of the alloys of this invention as well as prior art alloys showed less than 0.001 I.P.Y. attack in 70% nitric acid at 80° C. Results were similar in tests in 15% HNO<sub>3</sub> plus 15% H<sub>2</sub>SO<sub>4</sub>-water solutions.

TABLE VII

| ALLOY NUMBER | CORROSION RATE IN 25% H <sub>2</sub> SO <sub>4</sub> PLUS 10% HNO <sub>3</sub> PLUS 4 OUNCES/GAL. NaCl AT 80° C. | LOSS IN INCHES OF PENETRATION PER YEAR (I.P.Y.) |
|--------------|------------------------------------------------------------------------------------------------------------------|-------------------------------------------------|
|              | LOSS IN INCHES OF PENETRATION PER YEAR (I.P.Y.)                                                                  |                                                 |
| 1411         | 0.0007                                                                                                           |                                                 |
| 2215         | 0.0030                                                                                                           |                                                 |
| 2216         | 0.0006                                                                                                           |                                                 |
| 2226         | 0.0030                                                                                                           |                                                 |
| 2234         | 0.0029                                                                                                           |                                                 |
| 2235         | 0.0039                                                                                                           |                                                 |
| 2331         | 0.0008                                                                                                           |                                                 |

In view of the above it will be seen that the alloys of this invention not only resist the depassivating attack of salt water but also resist a wide variety of corrosive streams, some of them containing chloride contamination in themselves. They present a broad spectrum of corrosion resistance, particularly in moderately aggressive reducing or oxidizing conditions.

What is claimed is:

1. An air meltalbe, castable, fabricable, weldable, and non-magnetic alloy resistant to corrosion by chloride or other halide containing solutions, consisting essentially of between about 13.5% and about 29% by weight nickel, between about 23% and about 26% by weight

chromium, between about 3.75% and about 6% by weight molybdenum, between about 2.95% and 4.5% by weight manganese, between about 3% and 6.39% by weight copper, between about 0.3% and 2.07% by weight columbium (niobium), between about 0 and about 1.5% by weight silicon, between about 0 and about 0.09% by weight carbon, between about 0.10% and about 0.45% by weight nitrogen, up to about 1% by weight vanadium, up to about 1% by weight titanium, up to about 5% by weight cobalt, up to about 0.3% by weight of rare earth components selected from the group consisting of cerium, lanthanum, and misch metal, and between about 28% and 48% by weight iron, the sum of the nickel content and cobalt content being between about 18.5% and 29% by weight, and the nickel content exceeds the chromium content by between about 0.5% and about 6% by weight (basis, the entire alloy).

2. An alloy as set forth in claim 1 containing between about 24% and 29% by weight nickel, between about 23% and about 26% by weight chromium, between about 3.75% about and 6% by weight molybdenum, between about 3% and about 4.5% by weight copper, between 2.95% and 4.5% by weight manganese, between about 0.3% and about 2.07% by weight columbium, between about 0.10% and about 0.45% by weight nitrogen, between 0.10% and about 0.50% by weight silicon, and up to about 0.05% by weight carbon, the nickel content exceeding the chromium content by between about 0.5% and about 6% by weight (basis, the entire alloy).

3. An alloy as set forth in claim 1 containing between about 25% and about 29% by weight nickel, between 23% and about 26% by weight chromium, between about 4% and about 6% by weight molybdenum, between about 3% and about 4.5% by weight copper, between about 2.95% and about 4.5% by weight manganese, between 0.3% and about 1.5% by weight columbium, and between about 0.10% and about 0.25% by weight nitrogen, the nickel content exceeding the chromium content by between 2% and about 5% by weight (basis, the entire alloy).

4. An alloy as set forth in claim 1 containing between about 26% and about 29% by weight nickel, between 23% and about 26% by weight chromium, between about 4.5% and about 5.5% by weight molybdenum, between about 3% and about 4% by weight copper, between about 3% and about 4% by weight manganese, between 0.5 and about 1.0% by weight columbium, between 0.15% and about 0.25% by weight nitrogen, between 0.01% and about 0.04% by weight carbon, and between 0.10% and about 0.40% by weight silicon, the nickel content exceeding the chromium content by between 3% and about 5% by weight (basis, the entire alloy).

5. An air meltalbe, castable, fabricable, weldable, and non-magnetic alloy resistant to corrosion by chloride or other halide containing solutions, comprising approximately 27% by weight nickel, approximately 23% by weight chromium, approximately 5% by weight molybdenum, approximately 3% by weight copper, approximately 3.5% by weight manganese, approximately 0.8% by weight columbium, approximately 0.20% by weight nitrogen, approximately 0.30% by weight silicon, approximately 0.03% by weight carbon, and approximately 35% by weight iron.

\* \* \* \* \*